

Sept. 16, 1941.

K. KUMETAT ET AL

2,256,163

PHOTOGRAPHIC SILVER HALIDE EMULSION

Filed Dec. 23, 1939

Fig. 1.



SILVER HALIDE EMULSION SENSITIZED WITH THE PERCHLORATE OF THE COMPOUND DERIVED FROM 1,3,3-TRIMETHYLINDOLINE-2-METHENE- $\omega$ -ALDEHYDE AND 3-ETHYL-2-METHYL-1-(DIMETHYL-ETHYL-AMMONIUM-PROPYL)-5-CHLOROBENZIMIDAZOLIUM-ETHYLSULFATE.

Fig. 2.



SILVER HALIDE EMULSION SENSITIZED WITH THE PERCHLORATE OF THE COMPOUND DERIVED FROM 1,3,3,5-TETRAMETHYLINDOLINE-2-METHENE- $\omega$ -ALDEHYDE AND 3-ETHYL-2-METHYL-1-(DIMETHYL-ETHYL-AMMONIUM-PROPYL)-5-CHLOROBENZIMIDAZOLIUM-ETHYLSULFATE.

Fig. 3.



SILVER HALIDE EMULSION SENSITIZED WITH THE PERCHLORATE OF THE COMPOUND DERIVED FROM 1-ETHYL-BENZSELENAZOLINE-2-METHENE- $\omega$ -ALDEHYDE AND 3-ETHYL-2-METHYL-1-(DIMETHYL-ETHYL-AMMONIUM-PROPYL)-5-CHLOROBENZIMIDAZOLIUM-ETHYLSULFATE.

Fig. 4.



SILVER HALIDE EMULSION SENSITIZED WITH THE PERCHLORATE OF THE COMPOUND DERIVED FROM 1-ETHYL-THIAZOLIDINE-2-METHENE- $\omega$ -ALDEHYDE AND 2,3-DIMETHYL-1-(TRIMETHYLAMMONIUM-PROPYL)-5-CHLOROBENZIMIDAZOLIUM-METHYLSULFATE.

Fig. 5.



SILVER HALIDE EMULSION SENSITIZED WITH THE PERCHLORATE OF THE COMPOUND DERIVED FROM 1,3,3-TRIMETHYLINDOLINE-2-METHENE- $\omega$ -ALDEHYDE AND 1-(DIMETHYL-ETHYL-AMMONIUM-PROPYL)-2-METHYL-3-ETHYL-5,6-DICHLOROBENZIMIDAZOLIUM-ETHYLSULFATE.

Fig. 6.



SILVER HALIDE EMULSION SENSITIZED WITH THE PERCHLORATE OF THE COMPOUND DERIVED FROM 1,3,3,5-TETRAMETHYLINDOLINE-2-METHENE- $\omega$ -ALDEHYDE AND 1-(DIMETHYL-ETHYL-AMMONIUM-PROPYL)-2-METHYL-3-ETHYL-6,7-DICHLOROBENZIMIDAZOLIUM-ETHYLSULFATE.

INVENTORS

KARL KUMETAT  
GUSTAV WILMANNS

BY *Art, al John*

THEIR ATTORNEYS

Patented Sept. 16, 1941

2,256,163

# UNITED STATES PATENT OFFICE

2,256,163

## PHOTOGRAPHIC SILVER HALIDE EMULSION

Karl Kumetat and Gustav Wilmanns, Wolfen, Kreis Bitterfeld, Germany, assignors to General Aniline & Film Corporation, New York, N. Y., a corporation of Delaware

Application December 23, 1939, Serial No. 310,826  
In Germany December 24, 1938

4 Claims. (Cl. 95—7)

The present invention relates to photographic silver halide emulsions.

In U. S. patent application Ser. No. 234,604, filed October 12, 1938, we have described, together with Oskar Riester, silver halide gelatine emulsions sensitized with sensitizing dyes, which on one or both sides of the trimethine chain contain an alkylated benzimidazole ring.

Further investigation has shown, that silver halide gelatine emulsions of improved sensitizing properties are obtained by incorporating therein sensitizing dyes of the above group, in which the nitrogen atom of the benzimidazole ring is substituted by an alkyl radical containing a trialkylammonium group. In this trialkylammonium group the nitrogen is pentavalent, the dyes are accordingly dibasic in character and have the following constitution:



In this formula  $n$  is a whole number greater than 1 and  $R_1$ ,  $R_2$ ,  $R_3$  the same or different alkyl radicals.  $X$  is an anion and the dotted line connecting the 2 carbon atoms of the right hand hetero radical indicates an atom grouping capable of completing the heterocyclic ring in the manner usual in cyanine dyestuff chemistry.

These dyes possess a greater water solubility and therefore yield photographic layers, which are not colored by a sensitizing dye after treatment in the photographic baths in an undesirable manner. They possess furthermore the same advantages compared with known dyestuffs as the sensitizers of the above named prior application.

The dyes are prepared according to the process described in U. S. patent application Ser. No. 237,475, filed October 28, 1938, assigned to the present assignee, by exchanging the quaternary  $N$ -alkyl-2-methylbenzimidazole for quaternary alkyl derivatives of  $N$ -(dialkylaminoalkyl)-2-methylbenzimidazole of the following formula:



The characters have the same meaning as in the preceding formula. This compound is first pre-

pared in its non-quaternary form as described in "Annalen" 394, page 65 for  $N$ -phenyl-2-methylbenzimidazole.

5

10

15

20

25

30

35

40

45

50

55

60



This compound is rendered quaternary with 2 mols of an alkyl acid ester.

The following examples when taken with the accompanying self-explanatory drawing, depicting the sensitivity of a number of emulsions sensitized with dyestuffs of the application serve to illustrate the invention:

### Example I

The dyestuff of 1,3,3-trimethylindoline-2-methene- $\omega$ -aldehyde and 2,3-dimethyl-1-(trimethylammonium-propyl)-5-chlorobenzimidazoliummethylsulfate is precipitated with 20% aqueous sodium perchlorate solution and has the following formula:



The dyes sensitize with a maximum at 535 m $\mu$ .  
Sensitizing range up to 560 m $\mu$ .

### Example II

The dye of 1,3,3-trimethylindoline-2-methene- $\omega$ -aldehyde and 3-ethyl-2-methyl-1-(dimethyl-ethyl-ammonium-propyl)-5-chlorobenzimidazolium-ethylsulfate is precipitated with 20% aqueous sodium perchlorate solution and has the following formula:



The dyes sensitize as shown in Figure 1 with a maximum at 535 m $\mu$ . Sensitizing range up to 560 m $\mu$ .

*Example III*

The dye of 1,3,3,5 - tetramethylindoline-2-methene- $\omega$ -aldehyde and 3-ethyl-2-methyl-1-(dimethyl-ethyl-ammonium-propyl)-5-chlorobenzimidazolium-ethylsulfate is precipitated with 20% aqueous sodium perchlorate solution and has the following formula:



The dyes sensitize as shown in Figure 2 with a maximum at 548 m $\mu$ . Sensitizing range up to 580 m $\mu$ .

*Example IV*

The dyestuff of 1-ethyl-benzselenazoline-2-methene- $\omega$ -aldehyde and 2,3-dimethyl-1-(trimethylammonium-propyl)-5-chlorobenzimidazolium-methylsulfate is precipitated with 20% aqueous sodium perchlorate solution and has the following formula:



The dyes sensitize with a maximum at 560 m $\mu$ . Sensitizing range up to 585 m $\mu$ .

*Example V*

The dye of 1-ethyl-benzselenazoline-2-methene- $\omega$ -aldehyde and 3-ethyl-2-methyl-1-(dimethyl-ethyl-ammonium-propyl)-5-chlorobenzimidazolium-ethylsulfate is precipitated with 20% aqueous sodium perchlorate solution and has the following formula:



The dyes sensitize as shown in Figure 3 with a maximum at 560 m $\mu$ . Sensitizing range up to 585 m $\mu$ .

*Example VI*

The dyestuff of 1-ethyl-thiazolidine-2-methene- $\omega$ -aldehyde and 2,3-dimethyl-1-(trimethylammonium-propyl)-5-chlorobenzimidazolium-methylsulfate is precipitated with 20% aqueous sodium perchlorate solution and has the following formula:



The dyes sensitize as shown in Figure 4 with a maximum at 500 m $\mu$ . Sensitizing range 450-525 m $\mu$ .

*Example VII*

The dye of 1-ethyl-thiazolidine-2-methene- $\omega$ -aldehyde and 3-ethyl-2-methyl-1-(dimethyl-ethyl-ammonium-propyl)-5-chlorobenzimidazolium-ethylsulfate is precipitated with 20% aqueous sodium perchlorate solution and has the following formula:



The dyes sensitize with a maximum at 500 m $\mu$ . Sensitizing range 450-525 m $\mu$ .

*Example VIII*

The dyestuff of 1-ethyl-thiazolidine-2-methene- $\omega$ -aldehyde and 2,3-dimethyl-1-(trimethylammonium-propyl)-benzimidazolium-methylsulfate is precipitated with 20% aqueous sodium perchlorate solution and has the following formula:



The dyes sensitize with a maximum at 495 m $\mu$ . Sensitizing range 450-515 m $\mu$ .

*Example IX*

The dye of 1-ethyl-benzselenazoline-2-methene- $\omega$ -aldehyde and 2,3-dimethyl-1-(trimethylammonium-propyl)-benzimidazolium-methylsulfate is precipitated with 20% aqueous sodium

perchlorate solution and has the following formula:



The dyes sensitize with a maximum at 555 m $\mu$ .  
Sensitizing range up to 580 m $\mu$ .

**Example X**

The dye of 1-ethyl-thiazolidine-2-methene- $\omega$ -aldehyde and 2,3,6-trimethyl-1-(trimethylammonium-propyl)-5-chlorobenzimidazolium-methylsulfate is precipitated with 20% aqueous sodium perchlorate and has the following formula:



The dyes sensitize with a maximum at 500 m $\mu$ .  
Sensitizing range 450-520 m $\mu$ .

**Example XI**

The dye of 1-ethyl-thiazolidine-2-methene- $\omega$ -aldehyde and 2,6-dimethyl-3-ethyl-1-(dimethyl-ethyl-ammonium-propyl)-5-chlorobenzimidazolium-ethylsulfate is precipitated with 20% aqueous sodium perchlorate and has the following formula:



The dyes sensitize with a maximum at 500 m $\mu$ .  
Sensitizing range 450-520 m $\mu$ .

**Example XII**

The dyestuff of 1-ethyl-thiazolidine-2-methene- $\omega$ -aldehyde and 2,3-dimethyl-1-(trimethylammonium-propyl)-5,6-dichlorobenzimidazolium-methylsulfate is precipitated with 20% aqueous sodium perchlorate and has the following formula:



The dyes sensitize with a maximum at 510 m $\mu$ .  
Sensitizing range 450-530 m $\mu$ .

**Example XIII**

The dye of 1-ethyl-thiazolidine-2-methene- $\omega$ -aldehyde and 2,3-dimethyl-1-(trimethylammonium-propyl)-6-chlorobenzimidazolium-methyl-

sulfate is precipitated with 20% aqueous sodium perchlorate and has the following formula:



The dyes sensitize with a maximum at 500 m $\mu$ .  
Sensitizing range 450-520 m $\mu$ .

**Example XIV**

The dye of 1-ethyl-thiazolidine-2-methene- $\omega$ -aldehyde and 2,3,5-trimethyl-1-(trimethylammonium-propyl)-6-chlorobenzimidazolium-methylsulfate is precipitated with 20% aqueous sodium perchlorate and has the following formula:



The dyes sensitize with a maximum at 500 m $\mu$ .  
Sensitizing range 450-520 m $\mu$ .

**Example XV**

The dyestuff of 1-ethyl-thiazolidine-2-methene- $\omega$ -aldehyde and 1-(dimethyl-ethylammonium-propyl)-2-methyl-3-ethyl-5-chloro-6-isopropyl-benzimidazolium-ethylsulfate is precipitated with 20% aqueous sodium perchlorate and has the following formula:



The dyes sensitize with a maximum at 500 m $\mu$ .  
Sensitizing range 450-520 m $\mu$ .

**Example XVI**

The dye of 1-ethyl-thiazolidine-2-methene- $\omega$ -aldehyde and 2,3-dimethyl-1-(trimethylammonium-propyl)-6,7-dichlorobenzimidazolium-methylsulfate is precipitated with 20% aqueous sodium perchlorate and has the following formula:



The dyes sensitize with a maximum at 500 m $\mu$ .  
Sensitizing range 450-520 m $\mu$ .

**Example XVII**

The dye of 1-ethyl-thiazolidine-2-methene- $\omega$ -aldehyde and 2,3-dimethyl-1-(trimethylammonium-propyl)-5-trifluormethyl-benzimidazolium-methylsulfate is precipitated with 20%

aqueous sodium perchlorate and has the following formula:



The dyes sensitize with a maximum at 500 m $\mu$ . Sensitizing range 450-520 m $\mu$ .

*Example XVIII*

The dyestuff of 1,3,3-trimethylindoline-2-methene- $\omega$ -aldehyde and 1-(dimethyl-ethyl-ammonium-propyl)-2-methyl-3-ethyl-5,6-dichlorobenzimidazolium-ethylsulfate is precipitated with 20% aqueous sodium perchlorate and has the following formula:



The dyes sensitize as shown in Figure 5 with a maximum at 555 m $\mu$ . Sensitizing range up to 30 580 m $\mu$ .

*Example XIX*

The dye of 1,3,3-trimethylindoline-2-methene- $\omega$ -aldehyde and 1-(dimethyl-ethylammonium-propyl)-2,5-dimethyl-3-ethyl-6-chlorobenzimidazolium-ethylsulfate is precipitated with 20% aqueous sodium perchlorate and has the following formula:



The dyes sensitize with a maximum at 545 m $\mu$ . Sensitizing range up to 570 m $\mu$ .

*Example XX*

The dye of 1,3,3,5-tetramethylindoline-2-methene- $\omega$ -aldehyde and 1-(dimethyl-ethyl-ammonium-propyl)-2-methyl-3-ethyl-5,6-dichlorobenzimidazolium-ethylsulfate is precipitated with 20% aqueous sodium perchlorate and has the following formula:



The dyes sensitize with a maximum at 565 m $\mu$ . Sensitizing range up to 590 m $\mu$ .

*Example XXI*

The dyestuff of 1-ethyl-thiazolidine-2-methene- $\omega$ -aldehyde and 1-(trimethylammonium-propyl)-2,3,4-trimethyl-benzimidazolium-methylsulfate is precipitated with 20% aqueous

sodium perchlorate and has the following formula:



The dyes sensitize with a maximum at 495 m $\mu$ . Sensitizing range 450-515 m $\mu$ .

*Example XXII*

The dye of 1-ethyl-thiazolidine-2-methene- $\omega$ -aldehyde and 1-(trimethylammonium-propyl)-2,3,5-trimethyl-benzimidazolium-methylsulfate is precipitated with 20% aqueous sodium perchlorate and has the following formula:



The dyes sensitize with a maximum at 500 m $\mu$ . Sensitizing range 450-520 m $\mu$ .

*Example XXIII*

The dye of 1,3,3-trimethylindoline-2-methene- $\omega$ -aldehyde and 1-(dimethyl-ethyl-ammonium-propyl)-2-methyl-3-ethyl-6,7-dichlorobenzimidazolium-ethylsulfate is precipitated with 20% aqueous sodium perchlorate and has the following formula:



The dyes sensitize with a maximum at 550 m $\mu$ . Sensitizing range up to 575 m $\mu$ .

*Example XXIV*

The dyestuff of 1,3,3,5-tetramethyl-indoline-2-methene- $\omega$ -aldehyde and 1-(dimethyl-ethyl-ammonium-propyl)-2-methyl-3-ethyl-6,7-dichlorobenzimidazolium-ethylsulfate is precipitated with 20% aqueous sodium perchlorate and has the following formula:



The dyes sensitize as shown in Figure 6 with a maximum at 560 m $\mu$ . Sensitizing range up to 585 m $\mu$ .

The dyes are added either directly to the emulsions in the usual concentration or they may be incorporated in the emulsion by bathing the same in a solution of the dye. The dyes may also be employed in mixture with other carbocya-

nines. Especially mixtures with orthochromatically sensitizing dyes such as pseudocyanines are useful.

We claim:

1. A silver halide gelatine emulsion containing an unsymmetrical benzimidazole trimethine cyanine dye in which one of the nitrogen atom of the benzimidazole nucleus carries the radical



$n$  being a whole number greater than 1 and  $\text{R}_1, \text{R}_2, \text{R}_3$  being alkyl.

2. A silver halide gelatin emulsion containing a dyestuff corresponding to the following formula:



wherein  $\text{R}_1, \text{R}_2, \text{R}_3$  is alkyl,  $\text{X}$  is an acid radical and  $n$  is a whole number greater than 1.

3. A silver halide gelatine emulsion containing

a dyestuff corresponding to the following formula:



wherein  $\text{R}_1, \text{R}_2, \text{R}_3$  is alkyl,  $\text{X}$  is an acid radical and  $n$  is a whole number greater than 1.

4. A silver halide gelatin emulsion containing a dyestuff corresponding to the following formula:



wherein  $\text{R}_1, \text{R}_2, \text{R}_3$  is alkyl,  $\text{X}$  is an acid radical and  $n$  is a whole number greater than 1.

KARL KUMETAT.  
GUSTAV WILMANNS.